

# United States Patent Office.

GEORGE JAMES HINDE, OF WOLVERHAMPTON, ENGLAND.

*Letters Patent No. 94,492, dated September 7, 1869; patented in England, February 26, 1869.*

## IMPROVEMENT IN COATING IRON OR STEEL WITH COPPER OR BRASS, OR OTHER ALLOYS OF COPPER.

The Schedule referred to in these Letters Patent and making part of the same.

To all to whom it may concern:

Be it known that I, GEORGE JAMES HINDE, of Wolverhampton, in the county of Stafford, England, manager of works, a subject of the Queen of Great Britain, have invented or discovered certain new and useful "Improvements in Coating Iron or Steel with Copper or Brass, or other Alloys of Copper;" and I, the said GEORGE JAMES HINDE, do hereby declare the nature of the said invention, and in what manner the same is to be performed, to be particularly described and ascertained in and by the following statement thereof; that is to say—

My invention consists of the improvements herein-described, in coating iron or steel with copper or brass, or alloys of copper, by which improvements the coating of the iron and steel is effected at a comparatively low temperature, and the difficulties which occur from the high temperature ordinarily required for effecting the said coating are avoided.

My invention is especially applicable to the coating of sheets of iron and steel with copper or brass, or certain other alloys of copper, but is also applicable to the coating of various articles of iron or steel, either in a manufactured or partly-manufactured state, such as wire, bars, or rods, tubes, or vessels.

My invention is especially applicable to the coating of iron or steel with copper or brass, or alloy of copper and zinc, but is also applicable to the coating of iron or steel with copper alloyed with other metals than zinc, such as an alloy of copper with tin or with lead.

I will describe my invention, with reference to the coating of iron or steel with copper or brass.

I clean the sheets or articles to be coated by any of the well-known pickling or other processes ordinarily employed for that purpose, and I plunge the sheets or articles into a bath of melted zinc, containing copper in alloy with the said zinc, the quantity of zinc being so large, compared with that of the copper, as not to materially affect the color of the zinc. From five to six parts, by weight, of zinc, to one part, by weight, of copper, I find to answer well in practice, but I do not limit myself to these proportions.

After a short immersion of the iron or steel sheets or articles in the said bath, they are withdrawn and exposed to heat in a muffle or heating-chamber, sufficiently hot to volatilize the zinc, and the sheets or articles are allowed to remain in the said muffle or heating-chamber until so much of the zinc has been volatilized as to leave brass upon the sheets or articles, or when a coating of copper is required, the sheets or articles are allowed to remain in the muffle or heating-chamber until the whole, or nearly the whole of the zinc has been volatilized.

In order to prevent the sheets or articles from ad-

hering together, or receiving any injury to their coating, I prefer, before putting them in the muffle or heating-chamber, to coat them with a mixture of finely-ground calcined flint and water. This coating, when dry, protects the surface of the metal, and does not prevent the volatilization of the zinc.

After the sheets or articles are removed from the muffle or heating-chamber, the coating of powdered flint is removed.

The articles are finished by burnishing or otherwise, and I prefer to pass the sheets that have been coated according to my invention, through a pair of plain rolls, in order to give smoothness to the coating.

Instead of proceeding in the manner described, the sheets or articles to be coated with copper or brass may first receive a coating of zinc, by the ordinary galvanizing-process, or they may be coated with tin or terne metal before being plunged into the bath of zinc and copper. A coating of copper alloyed with tin, or an easily-fused metal other than zinc, may be applied to sheets and articles of iron or steel, by a process similar to that already described, excepting that tin, or the other easily-fused metal, is to be employed in addition to the zinc.

Having explained generally the nature of my invention, I will proceed to describe more in detail the manner in which the same is to be carried into effect.

For convenience of description, I will describe my invention as applied to the coating of iron, although it must be understood that both wrought and cast, and malleable cast-iron and steel may be coated with copper, brass, or other alloy of copper, by my invention.

I first make the surface of the iron to be coated perfectly clean. This I effect either by the process called pickling, that is, immersion of the iron in dilute sulphuric acid or muriatic acid, a process well understood and commonly practised, or by mechanical abrasion of the surface by scouring, filing, turning, or other mechanical operation.

I prefer to dip the cleaned iron into a solution of sal-ammoniac before proceeding to coat it with the alloy of copper. The iron, on removal from the said solution, is coated with a thin film of sal-ammoniac. A solution of one pound of sal-ammoniac to one quart of water, answers very well for this purpose, but other proportions may be employed.

In making a bath of melted zinc and copper, which I will hereinafter call the coating-bath, I melt one part, by weight, of copper, in a crucible or melting-pot, and add thereto five parts, by weight, of zinc. The melted metals, on being stirred, immediately form an alloy, and the coating of the iron may be effected by plunging it, prepared in the manner hereinbefore described, into the melted alloy contained in the cruci-

ble or melting-pot in which it is made. I prefer, however, to transfer the melted alloy into a bath or vessel, similar to that used for galvanizing iron, set in a furnace, and heated to a temperature sufficient to keep the alloy in a state of perfect fusion.

Before immersing the iron to be coated into this coating-bath, I prefer to throw some sal-ammoniac on the surface of the coating-bath, and to introduce the iron to be coated through the layer of sal-ammoniac on the coating-bath. The iron, on being plunged into and withdrawn from the coating-bath, will be found to have received a coating of the alloy.

The quantity of sal-ammoniac which I prefer to throw on the surface of the coating-bath, previous to the immersion of the iron, varies from a few ounces to a few pounds, according to the size of the iron to be coated. As the said sal-ammoniac volatilizes rapidly at the temperature of the coating-bath, I prefer to add it to the bath immediately before the immersion of the iron therein.

I also add zinc to the coating-bath from time to time, in order to replace that lost by volatilizing.

Although for ordinary purposes I effect the coating in a manner already described, yet the said coating may be effected upon iron, which has previously received a coating of zinc, or of tin, or of tin and lead, commonly called terne metal.

In coating, according to my invention, iron which has received a preliminary coating of zinc or tin or terne metal, I proceed in the manner already described, excepting that the cleaning and immersion in a solution of sal-ammoniac are unnecessary.

When the iron has received a preliminary coating of tin or terne metal, the composition of the coating-bath is liable to be affected thereby, the coating-bath becoming charged more or less with tin or tin and lead, and the proportion of copper relatively diminished. In such cases, I add to the coating-bath from time to time small portions of melted copper or of brass, in addition to the zinc added from time to time, so as to keep the proportion of copper in the bath, as nearly as may be, the proportion of one part of copper to five parts of zinc, or the other metal or metals.

Where it is wished to coat the iron with an alloy of copper and tin, or copper and terne metal, I coat the iron first with tin or with terne metal, in the ordinary manner, and I plunge it into and quickly withdraw it from the coating-bath.

In this way, the iron is coated with the alloy of zinc and copper upon the coating of tin or terne metal, more or less of the said coating of tin or terne metal being removed from the iron during its immersion in the coating-bath. Or I add the required amount of tin or terne metal to the coating-bath, and introduce the uncoated iron therein in the same manner as when a coating of copper or brass is to be given to the iron. I prefer, however, in all cases where practicable, to use iron with no preliminary coating, and to make the coating-bath of the exact composition which it is wished the coating to be given to the iron shall have previous to the heating-process hereinafter described.

The preliminary coating of zinc, or tin, or terne metal, is principally useful where small articles or articles of complex form are to be coated with copper or alloy of copper. In such cases there is no risk of the coating failing in any part through oxidation of the iron or steel, as sometimes happens when the iron or steel has not received a preliminary coating.

The iron, after immersion and removal from the coating-bath, is coated with a thin coating of the zinc and copper alloy, or when the iron has been previously coated with tin or with terne metal, the coating contains, besides zinc and copper, a portion of tin or terne metal. The coating on the iron, after removal from the coating-bath, much resembles a coating of zinc,

being of a nearly white color, and giving little or no indication by its color of the presence of copper. I will hereinafter call the iron in this stage alloy-coated iron.

I next proceed to volatilize so much of the zinc of the alloy-coated iron as to produce a coating of brass or copper, or copper more or less alloyed with zinc, in the following manner: I place, in a vessel of convenient size and shape, a mixture of ground calcined flint and water, mixed to about the consistency of cream, and I immerse the alloy-coated iron in the said mixture, and immediately withdraw it therefrom. A coating of flint and water adheres to the said iron. This coating is quickly dried by the application of heat on or in a stove or in any other convenient manner. The alloy-coated iron, thus coated with dried calcined ground flint, is then placed in a conveniently-shaped annealing-box or vessel of iron or other refractory material. The alloy-coated iron, placed in the annealing-box or vessel, is covered by another box or vessel, somewhat smaller, but of the same shape, inverted in the larger box or vessel, the space between the sides of the smaller box or vessel and those of the larger box or vessel being filled with dried calcined powdered flint. The box or vessel containing the alloy-coated iron is then placed in an annealing-muffle, and heated until it is at a bright-red heat throughout. About twenty to thirty minutes' exposure to this heat is usually sufficient to volatilize so much of the zinc of the alloy-coated iron that an alloy of copper and zinc, in the proportions in which they form brass, is left on the iron. By prolonging the time of exposure to heat, more zinc is volatilized, until eventually the whole or nearly the whole of the zinc is driven off, and a coating of pure or nearly pure copper is left on the iron. To volatilize the whole or nearly the whole of the zinc, about two hours' exposure of the alloy-coated iron at a bright-red heat is usually sufficient. Where large annealing-boxes are employed, a longer exposure to heat is required, and where a very high temperature is employed, the zinc is volatilized more rapidly.

If the iron that has been coated is in the form of bars, rods, or plates, and it is desired to have a smoother surface than it has when taken from the muffle, or heating-chamber, it is passed through rolls, the adhering ground calcined flint having been previously washed or brushed off. The iron may be softened, if required, after being rolled, by subjecting it to a dull-red heat. The coated iron is then scoured with sand and water, and rapidly dried by heat, in or on a stove or other means.

When manufactured or partly-manufactured articles are coated by my invention, and it is wished to make the coated surface smooth, this is effected by the process of burnishing, planishing, spinning, or other mechanical treatment, as is well understood.

When wire has been coated according to my invention, it may be drawn in the same manner as brass wire is drawn, and annealed during the drawing-process. If the wire is to be worked into manufactured articles in a hard state, it must not be annealed after the final drawing, but if it is required to be used in a softened state, it must be annealed after the final drawing.

By using the proportion of zinc to copper in the coating-bath hereinbefore described, or thereabout, I avoid many difficulties that arise in attempting to coat iron with copper or brass directly, as the mixture of copper and zinc that I use is very fusible, and can be kept melted by the application of heat in an iron vessel, in the same manner as molten zinc.

By the use of a coating of powdered flint to the alloy-coated iron, previous to the volatilization of the zinc, the surfaces of the coated iron are prevented from touching each other in the pans or vessels, and the coated surface is less oxidized or tarnished than

94 492

21.92

3

when the alloy-coated iron is without the coating of powdered flint.

Although I prefer to use calcined powdered flint for the purpose described, yet I do not limit myself thereto, as other finely-divided substances may be employed; and although I prefer to give the alloy-coated iron a coating of powdered flint or other matter previous to introducing it into the muffle, or heating-chamber, yet the use of the said coating of powdered flint or other matter may be dispensed with in carrying my invention into effect, and other methods resorted to of keeping the sheets or articles apart during the volatilization of the zinc.

Having now described the nature of my invention, and the manner in which the same is to be performed, I wish it to be understood that I do not limit myself to the precise details herein described, as the same may be varied without departing from the nature of my invention; but

I claim as my invention—

The improvements hereinbefore described in coating iron or steel with copper or brass or other alloys of copper, that is to say, coating iron or steel with copper or brass, by giving to the said iron or steel a coat-

ing of an alloy of copper and zinc, the proportion of zinc in the said alloy being so great that the said alloy differs but little in fusibility and other physical characteristics from zinc, and afterward volatilizing, by heat, the zinc of the said alloy, either wholly or in part, and thereby leaving upon the said iron or steel a coating of copper or brass, substantially as described.

Also, the modifications described with reference to the coating of iron or steel, previously coated with tin or terne metal, and the modifications described, when it is wished that the final coating shall contain, in addition to copper or copper and zinc, tin or terne metal.

Further, the use of a film of powdered calcined flint or other finely-divided substance, for protecting the alloy-coated iron or steel from injury and oxidation during the volatilization of the zinc or other volatile metal contained in the coating.

GEORGE JAMES HINDE. [L. S.]

Witnesses:

GEORGE SHAW,  
7 Cannon Street, Birmingham.  
RICHARD SKERRITT,  
7 Cannon Street, Birmingham.